

## UNITED STATES PATENT OFFICE

FREDERICK ARTHUR HILL, OF EALING, LONDON, ENGLAND

## LIQUID COMPOSITION FOR PRESERVING MATERIALS, PARTICULARLY TIMBER

No Drawing. Application filed May 15, 1930, Serial No. 452,816, and in Great Britain March 14, 1930.

This invention comprises improvements in or relating to liquid compositions for preserving materials particularly timber.

Creosote is used in large quantities for preserving railway sleepers and other timber, and one object of the present invention is to provide a substitute for creosote which shall be less expensive but nevertheless substantially as effective as regards its preservative properties.

The composition provided according to this invention comprises a mixture of crude oil, bituminous material, and a small proportion of naphthalene or other preservative adapted to prevent insect attack.

Preferably the basis of the composition is fuel oil (otherwise known as Diesel oil) that is to say, the petroleum product from which the lighter constituents such as naphtha and the greater part of the illuminating oils and kerosenes have been separated.

The term "bituminous material" is used to include natural and artificial asphalt, tar, pitch and the like and also mixtures of these substances. Preferably in carrying out the invention bitumen of the type artificially prepared from petroleum, such as Mexican asphalt, is employed.

In one example according to the invention the composition was prepared in the following way. Mexican asphalt was first liquefied by heat and there was then mixed with the molten asphalt a proportion of liquid naphthalene prepared by melting crystals. The molten mixture of bitumen and naphthalene was then added to a main body of fuel oil and thoroughly incorporated therewith by agitation in a mixer. The resulting composition contained 85% fuel oil, 10% asphalt and 5% naphthalene.

The proportions given above may be varied within comparatively wide limits without departing from the scope of the invention. One function of the bitumen is to act as a pore-filling material, and the proportion of bitumen in the composition will naturally vary with the nature of the timber to be treated. For example with a soft wood it may be desirable to have a comparatively high proportion of bitumen in the composi-

tion. One function of the naphthalene is to prevent insect attack, another is to render the bitumen more readily miscible with the oil. It will usually be desirable therefore to accompany any increase in the proportion of bitumen with a corresponding increase in the proportion of the naphthalene.

Some crude oils have as a natural constituent a substantial bitumen content. When such oils are employed in the present invention, it might not be necessary to add a further proportion of bitumen, and in any case the proportion of added bitumen would be less than the case where fuel oil is used.

One advantage of this invention is that, on account of the part played by the bitumen, the cheaper and softer woods, which have hitherto been found unsatisfactory for the manufacture of railway sleepers, may now be used for that purpose.

## I claim:

A process for the manufacture of a liquid composition for preserving timber which consists in preparing a molten mixture of asphalt and naphthalene in the proportions of about 2 parts asphalt to 1 part of naphthalene, and thoroughly incorporating this mixture with a main body of fuel oil in proportions of about 15 parts asphalt-naphthalene mixture to 85 parts fuel oil.

In testimony whereof I affix my signature.

FREDERICK ARTHUR HILL.

85

90

95

100